

Feb. 27, 1951

E. H. LAND ET AL

2,543,179

DEVELOPER FOR DICHROIC IODINE IMAGES

Original Filed March 13, 1942



FIG. 2



FIG. 3



Edwin H. Land  
Joseph M. Mable  
and  
Mark Hyman Jr.  
INVENTORS

BY  
Donald L. Brown  
ATTORNEY

## UNITED STATES PATENT OFFICE

2,543,179

## DEVELOPER FOR DICHROIC IODINE IMAGES

Edwin H. Land, Cambridge, Joseph Mahler, Brookline, and Mark Hyman, Jr., Cambridge, Mass., assignors to Polaroid Corporation, Cambridge, Mass., a corporation of Delaware

Original application March 13, 1942, Serial No. 434,568. Divided and this application November 13, 1945, Serial No. 628,314.

6 Claims. (Cl. 95—88)

1

This invention relates to photography and more particularly has reference to a processing solution or developer, and especially an agent of this character which may be employed for the formation or development of an image in iodine.

This application is a division of our copending application, Serial No. 434,568, filed March 13, 1942, now abandoned, for Light Polarizers and Methods and Materials for Forming the Same.

Objects of the invention reside in the provision of photographic developers for treating an image comprising an oxidizing agent carried by photographic film, the developer being of a character which effects the replacement or conversion of the oxidizing image to a dichroic stain as well as a developer which reacts with an oxidizing agent of suitable oxidizing potential to cause the release of iodine from the developer.

Another object of the invention is to provide a photographic developer for forming dichroic or light-polarizing images in a transparent, molecularly oriented, linear polymeric plastic, for example, oriented polyvinyl alcohol, which has been rendered light sensitive and exposed to light, particularly molecularly oriented plastics which have been sensitized with dichromates.

A further object of the invention resides in the provision of a developer comprising an acid solution of one or more iodides to which may be added an agent adapted to harden or stiffen the material of which an image-carrying layer is formed, a reducing agent, a buffer for the acid and an agent adapted to control the color of the finished product.

The invention accordingly comprises the product possessing the features, properties and proportions of constituents, which are exemplified in the following detailed disclosure, and the scope of the application of which will be indicated in the claims.

For a fuller understanding of the nature and objects of the invention, reference should be had to the following detailed description taken in connection with the accompanying drawing, in which:

Figure 1 is a somewhat diagrammatic view illustrating a convenient arrangement for exposing the sensitive material of the invention to light during the printing from a photographic negative;

Fig. 2 is a diagrammatic view in perspective illustrating a print prepared in accordance with the invention as it appears when viewed without an analyzer; and

Fig. 3 is a similar view showing the same print as it appears when viewed through a suitable

2

analyzer having its polarizing axis at right angles to the polarizing axis of said print.

The process of the present invention comprises three main steps—treatment of a sheet of the desired material with a suitable photo-sensitizing material, exposure of the sensitized sheet to light, and treatment of the sheet with a developing agent adapted to produce a dichroic stain in the exposed areas thereof. In addition to these steps, it may be desirable in some cases to add a fourth step comprising treatment of the developed sheet in an intensifier bath. Particular novelty lies in the fact that the stain which constitutes the image is produced by reaction between the developing agent and the light-sensitive material in the exposed areas of the sheet, the exposed material comprising an oxidizing agent of sufficient oxidizing potential to effect the release of the dichroic stain.

Suitable sheet materials which may be used in the practice of the invention include plastics, particularly a plastic from the class consisting of the linear, hydrophilic polymers, such for example as polyvinyl alcohol, polyvinyl acetal and regenerated cellulose. Of the materials falling within this class, the preferred material is polyvinyl alcohol, and prints or images formed in suitably prepared sheets of that material possess the highest dichroism and hence are most suitable in the production of superimposed right and left eye stereoscopic images.

For best results, the molecules, at least on the surface of the plastic sheet, should be substantially oriented in a predetermined direction.

This may conveniently be accomplished by softening the sheet, as for example by subjecting it to heat, and then stretching or extending the sheet until suitable orientation of the molecules has been obtained. In the case of polyvinyl alcohol, a sheet formed by casting may be placed in condition for the formation of dichroic images therein by extending to from two to four or five times its length.

Several specific examples and formulae will now be given, but it is to be understood that they are intended to be illustrative only and are in no way to be construed as limiting the invention to the specific times, proportions or percentages given. It should, moreover, be particularly noted that many variations may be made in any of the steps of the invention, provided that said variations are compensated for in the other said steps, as will be described in more detail hereinafter.

By way of illustration, the invention will be described with reference to a sheet of polyvinyl alcohol, and it will be assumed that the molecules

therein have already been substantially oriented. The first step in the process is to render the sheet light-sensitive, and this may be done conveniently by imbibing the sheet in a solution containing the desired photo-sensitizing agent. Among the materials found suitable for this purpose, the preferred materials comprise dichromates, such for example as ammonium dichromate, potassium dichromate and sodium dichromate, with ammonium dichromate being particularly preferred for the reason that it is the most soluble.

The solvent for the photo-sensitizing agent may be simply water, but this is not wholly satisfactory for the reason that it tends to penetrate the sheet too rapidly and thus tends to soften it unduly. It is preferable, therefore, to add to the solution a liquid which is miscible therewith but is a non-solvent of the plastic as well as non-reactive with the other chemicals present, and which accordingly tends to slow penetration of the sheet and thus aid in maintaining its stiffness. Suitable examples include acetone, methanol and ethylene glycol, and the volume thereof used may vary anywhere up to approximately 99% of the total volume of solvent present.

The proportion of sensitizing agent to solvent may vary within a wide range, from as low as 1 to 2% to as high as 40% based on the volume of solvent, provided the variation is compensated for by variation of the time of treatment approximately inversely to the proportion of sensitizing agent. Said time of treatment may vary from a few seconds upward but should preferably continue only long enough to permit the solution to penetrate the surface of the sheet uniformly for a short distance, and in no case should the sheet be allowed to soak so long that it softens unduly. It has also been found desirable to add a wetting agent such, for example, as soap or the product sold as "Aerosol MA," a product of American Cyanamid and Chemical Corporation in order both to accelerate the sensitizing treatment and to promote uniform sensitization. Specific reference to the product "Aerosol MA" as dihexyl sodium sulfosuccinate may be found on page 11 of "Handbook of Material Trade Names," Zimmerman and Lavine, Industrial Research Service, Dover, New Hampshire, 1946.

A typical satisfactory formula for the sensitizing bath is as follows:

|                     |    |    |
|---------------------|----|----|
| Water               | cc | 75 |
| Acetone             | cc | 25 |
| Ammonium dichromate | gm | 16 |
| "Aerosol MA"        | gm | 1  |

With a solution of approximately the foregoing formula, a sufficient time of treatment will be about two to three minutes, and the sheet should then be taken from the solution and the excess liquid wiped off or otherwise removed from its surface.

The next step of the process is to expose the sensitized sheet to the action of light. If the process is to be used to form a dichroic image of a photographic negative or the like, the exposure should be through the negative to be reproduced, as for example in the manner indicated in Fig. 1, wherein sensitized sheet 10 is represented as mounted under a photographic negative 12 and exposed to light rays emanating from light source 14 provided with a conventional reflector 16. Light source 14 may emit primarily white light or primarily ultraviolet light, and the time of exposure may vary considerably, depending on the intensity of the light, the distance be-

tween it and the sheet, and the degree to which the sheet was sensitized, as pointed out above. If, for example, an R2 Photoflood bulb mounted approximately six inches from the surface of sheet 10 be used as the light source, a sheet sensitized as described above for two to three minutes should be sufficiently exposed in from forty to sixty seconds.

It should be noted that during the exposure, 10 and particularly in the case of exposure for a long period, it may be advisable to shield sheet 10 from the infrared rays emanating from the light source, as by means of a suitable filter 15. If it is desired to print by means of the ultraviolet rays emanating from source 14, element 15 should also include filtering material for visible light, and the exposure time should be increased to about five minutes, owing to the absorption of the ultraviolet light by negative 12.

The effect of the exposure of the sensitized sheet of the invention to light is to harden the surface of the sheet approximately proportionally to the degree of exposure. As will be seen from Fig. 1, the degree of exposure varies according to 25 the variations of density in negative 12, i. e., more light is transmitted by the lighter areas of the negative than by the darker areas. The result is that the surface of sheet 10 is hardened to a varying degree corresponding inversely to the 30 density of negative 12. In other words, where the negative is lightest, sheet 10 is most exposed and most hardened, and where the negative is darkest, sheet 10 is relatively unexposed and remains relatively soft.

The next step in this embodiment of the process 35 is to eliminate unexposed light-sensitive material from sheet 10. This may be done in the present example by a simple washing with water to remove the dichromate from the unhardened 40 areas of the sheet, and the time of washing varies more or less according to the degree of sensitizing and the time of exposure, the important factors being that all unexposed dichromate should be removed but that the washing should not continue so long that the highlights of the picture 45 are washed out or the exposed dichromate affected. It is for this reason that the sensitizing treatment is preferably confined to the surface of the sheet; the unexposed dichromate may then be removed in as short a time as possible. For a sheet sensitized and exposed as described above, the washing should be completed in approximately 50 two minutes, but it must be emphasized that this time is by no means critical and may be varied considerably without appreciably altering 55 the result.

The next step in the process is to treat the exposed and washed sheet with a developing compound adapted to react with the light-sensitive 60 material in the exposed and hardened areas thereof to produce a dichroic stain. In the embodiment of the invention utilizing dichromate as the light-sensitive material, the developing compound comprises essentially an iodide solution of such characteristics and properties that it reacts with the dichromate in the sheet to produce the desired dichroic stain. In order to produce this reaction, the iodide or iodides used 65 should be water-soluble and in addition should be easily oxidizable by the dichromate.

These characteristics in the developer may 70 conveniently be secured either by using an alkali iodide, particularly ammonium iodide or an alkali metal iodide such, for example, as potassium iodide or sodium iodide, and adding one or more

acids to the solution, by using a solution of an iodide which is naturally easily oxidizable such, for example, as ferrous iodide or cerous iodide, or by using an iodide solution which is naturally acidic such, for example, as hydriodic acid. Preferred acids for use in the first case include hydrochloric and hydrobromic. Alternatively, any strong oxidizing acid such, for example, as sulphuric, nitric or phosphoric, or an organic acid such as acetic may be used.

It has already been pointed out that the result of the exposure step illustrated in Fig. 1 is to harden the surface of the sensitized sheet differentially, depending upon the optical density of the photographic negative at any given point. It follows, therefore, that after the exposed sheet has been washed, the amount of dichromate remaining therein will similarly vary differentially over its entire area. Then when the sheet is subjected to the developing treatment, the iodine stain absorbed in any particular area will depend upon the amount of dichromate present in that area. That is to say, the stain will be relatively intense in the areas where there is considerable dichromate, namely, the areas corresponding to light areas in the original negative. Conversely, there will be relatively little dichromate in the areas corresponding to the dark areas in the negative, and the amount of stain absorbed therein will therefore be substantially less. In other words, the final product of the developing step of the operation will be a positive reproduction in light-polarizing areas of the original negative image represented by element 12 in Fig. 1.

As is the case with the other compounds and steps of this invention, the composition of the developing solution may vary to a considerable extent, depending both on the results desired and on the way in which the preceding steps were carried out. For example, if the sheet was sensitized in a concentrated solution and exposed for a relatively long period, a concentrated developer may be used, but if the sheet was sensitized in a dilute solution and exposed for a short time, the developer and developing time must be correspondingly modified. Similarly, the particular acid used affects the developing time, a developer containing a strong acid like hydrochloric requiring a shorter time than one containing a weak acid like acetic. Several examples and formulae will be given, therefore, but it is to be understood that they are intended as illustrative only and the percentages and proportions therein are in no sense to be considered as critical.

A typical developer may be made up as follows:

|                         |    |      |
|-------------------------|----|------|
| Water                   | cc | 1000 |
| Acetone                 | cc | 80   |
| Hydrochloric acid (38%) | cc | 1.5  |
| Ammonium iodide         | gm | 11.6 |
| Potassium iodide        | gm | 1.6  |
| Boric acid              | gm | 9.2  |

The acetone in the above formula is used for the same purpose as in the sensitizing bath, namely, to maintain the stiffness of the sheet by preventing over-penetration by the solvent. As explained above, any similarly acting agent may be substituted therefor, and the percentage thereof is optional and merely approximate. It has been found that the mixed iodides appear to give better results than either alone, but either may be used alone, and it will be noted that the total amount thereof should preferably be about 1%. Said percentage, however, is by no means critical. On the contrary, it is possible to vary the iodide

content from as low as 5% up to the saturation point, about 40%.

The hydrochloric acid content in the developing solution should be kept relatively low, for otherwise it tends to attack and destroy the dichromate in the sheet. If, however, an oxidizing acid such as sulphuric or nitric is substituted for the hydrochloric, the amount thereof may be substantially higher. The boric acid appears to aid in controlling the color of the finished print.

A sheet sensitized and exposed as described above will be sufficiently developed after about one minute in a developer of approximately the above formula, and the resulting print will have relatively even characteristics and shading. If a more contrasty print is desired, it may be obtained by adding to the developer a suitable reducing agent, which will suppress any free iodine in the solution and remove or destroy any stain accidentally produced thereby in the unexposed areas of the sheet, thus lightening the light areas in the print and so increasing its contrast. It is also desirable to add to the developer a weak alkali, which will act as a buffer for the acid and thus aid in keeping uniform the action of the developer by maintaining the pH value thereof relatively constant.

Either a reducing agent or an alkali or both together may be used for the above purposes, and a suitable compound for use in this connection is the photographic developer sold as "DK-60," a product of Eastman Kodak Company, which will act both as an alkali and as a reducing agent. The amount of this compound which should be added to the developer depends largely on the degree of contrast desired in the prints, but in general it may be stated that satisfactory results are obtained by using approximately the following illustrative formula:

|                  |    |      |
|------------------|----|------|
| Water            | cc | 1000 |
| Acetone          | cc | 100  |
| HCl (38%)        | cc | 2    |
| Ammonium iodide  | gm | 10   |
| Potassium iodide | gm | 2    |
| Boric acid       | gm | 10   |
| "DK-60"          | cc | 40   |

"DK-60" is a silver halide developer well known to the art and specific reference thereto will be found in the handbook entitled "Photographic Chemicals and Solutions," Crabtree and Matthews, American Photographic Publishing Company, Boston, Massachusetts, 1938, on page 290, and under the heading "(DK-60)."

As in the preceding case, a sheet sensitized and exposed as described above should be sufficiently developed in the above developer in about one minute. If desired, however, the degree of contrast may be increased by then treating the sheet in an intensifying solution containing a reducing agent and preferably also a weak alkali. This treatment will further bleach and clear up the light areas, but care must be taken not to continue it so long that the highlights or other areas are affected. Ordinarily a minute should be sufficient, and a suitable illustrative formula for such a bath is as follows:

|                  |    |     |
|------------------|----|-----|
| Water            | cc | 160 |
| Acetone          | cc | 25  |
| HCl (38%)        | cc | 5   |
| Boric acid       | gm | 2   |
| Potassium iodide | gm | 45  |
| "DK-60"          | cc | 15  |

When the foregoing steps are completed, the print need only be wiped or otherwise dried and will then be finished. It will have approximately the appearance illustrated in Fig. 2, wherein print 20 bears a positive reproduction in dichroic areas of the image of negative 12, but the image will be relatively faint when viewed as in Fig. 2 without an analyzer. This is due to the fact that print 20, speaking in terms of optics, is merely an imperfect polarizer, which absorbs some of the light vibrating in one direction proportionally to the variations in density of its stained areas, but transmits the remainder of that component and all of the component vibrating in the opposite direction. In order, therefore, to see the image 10 thereon properly, it should be viewed through a suitable crossed analyzer.

Such an arrangement is shown in Fig. 3, wherein a polarizing element 30 of uniform polarizing characteristics is shown superimposed on print 20, with its polarizing axis at right angles to that of the print, as indicated by arrows 25 and 35. The result is that analyzer 30 absorbs all of that component of the light which is freely transmitted by print 20. On the other hand, the analyzer transmits the other component of the light, which is the component differentially absorbed by the print, and will thus cause the image on print 20 to appear in as complete detail and with as high a degree of clarity as a photographic print of negative 12 produced by conventional photographic methods. Conversely, if analyzer 30 were rotated through 90 degrees with respect to print 20, it would then act to absorb the remainder of the component differentially absorbed by the print, with the result that the image would disappear and the combined elements would appear substantially uniformly transparent.

The process of the invention is well adapted to the production of dichroic stereoscopic images. For example, the image shown in Figs. 2 and 3 may be assumed to be one image of a stereoscopic pair. In that event the other image should be reproduced on a plastic sheet having its molecules oriented substantially at right angles to the direction of molecular orientation in sheet 20. The two sheets may then be superimposed with the images thereon in relative stereoscopic registry, and the resulting composite image will have a three-dimensional effect when viewed through proper polarizing viewing means in accordance, for example, with Patent No. 2,203,687.

The terms "dichroism" and "dichroic" as used herein and in the claims are intended to refer to the property of polarizing transmitted light by differential absorption according to vibration direction. It will be noted that in its simplest form the process of the invention may be practiced to produce a uniform dichroic light-polarizing sheet. This may be done, for example, by sensitizing a sheet of the desired molecularly oriented plastic, exposing the sheet uniformly to light, and then treating as described above to produce a uniform dichroic stain therein. It is to be understood that this and similar modifications of the process of the invention are to be construed as coming within the scope thereof.

It should be pointed out that it is not at all essential to the practice of this invention that the various steps of the process thereof be carried out continuously. For example, the sensitizing treatment may take place at an entirely different time from the remainder of the process. It should also be noted that these sheets are relatively low in light sensitivity, and that only mod-

erate care need be taken to protect them from exposure to extraneous light while carrying out the other steps of the process of the invention.

It should be understood that many types of images other than photographic negatives may be reproduced by this process, such for example as a negative or positive of any other partially light-transmitting type or an opaque object of which it is desired to make a silhouette. The invention is particularly adapted, for example, to the reproduction of stencils, drawings, half-tones, printed matter and the like. Negative 12 in Fig. 1 should be considered, therefore, as representative of any such similar medium which will differentially transmit or block light directed toward the sensitized sheet, and the reproductions therefrom made by the process of this invention will be positive reproductions, that is to say, the light values therein will be reversed with respect to said negative.

Although, as has already been pointed out, the process of the present invention is particularly adapted for the production of light-polarizing images, it is not limited thereto and may be used 25 to produce non-polarizing images. In this modification of the invention, it is necessary only that the step of molecular orientation of the plastic sheet be omitted. If the process is carried out with this modification, the product will be substantially non-polarizing, positive reproduction 30 of the original image comparable in substantially every respect with a positive print produced by conventional photographic technique.

As has been previously stated, the foregoing 35 description is merely illustrative of one or more operative forms of the process of the present invention. It must again be emphasized that each step therein is a variable, and that none of the ingredients, times or proportions given for any 40 step is critical except in so far as it may be made so by the other variables. Thus, in the sensitizing step, the time of treatment, sensitizing agent used, and the concentration of the solution are mutually dependent, and all must be 45 considered in determining the proper exposure time. The degree of sensitizing and the degree of exposure, as well as the type of print desired, are mutually important to the choice of developer, and all four are governing factors in determining 50 the developing time and the question of whether or not an intensifying bath should also be used. It follows, therefore, that great variation is possible and that virtually any degree thereof in one or more steps can be compensated for in the other steps. It is accordingly obvious that no set 55 rules can be given and that it would be difficult if not impossible even to set outside limits on the ranges of variation.

Since certain modifications in the product 60 which embodies the invention may be made without departing from its scope, it is intended that all matter contained in the foregoing description, or shown in the accompanying drawing shall be interpreted as illustrative and not in a limiting 65 sense.

What is claimed is:

1. A composition for developing light-exposed dichromate which forms an image in an image-carrying layer of a hydrophilic, molecularly oriented, linear high polymer whereby to transform the dichromate to a dichroic material comprising iodine, said developing composition comprising water, hydrochloric acid, at least one easily oxidizable, water-soluble iodide salt, and 70 an agent comprising boric acid for controlling

the color of the iodine image formed by development of said dichromate, and wherein said composition is proportioned so that the hydrochloric acid thereof is restricted to a quantity insufficient to destroy dichromate undergoing development while the boric acid is present in a quantity sufficient to exert a visible effect upon the color of the iodine image formed by development of said dichromate and the iodide salt is present in a concentration of from 0.5% to the saturation point of said composition.

2. A composition for developing light-exposed dichromate which forms an image in an image-carrying layer of a hydrophilic, molecularly oriented, linear high polymer whereby to transform the dichromate to a dichroic material comprising iodine, said developing composition comprising water, hydrochloric acid, at least one easily oxidizable, water-soluble iodide salt comprising ammonium iodide, and an agent comprising boric acid for controlling the color of the iodine image formed by development of said dichromate, and wherein said composition is proportioned so that the hydrochloric acid thereof is restricted to a quantity insufficient to destroy dichromate undergoing development while the boric acid is present in a quantity sufficient to exert a visible effect upon the color of the iodine image formed by development of said dichromate and the iodide salt is present in a concentration of from 0.5% to the saturation point of said composition.

3. A composition for developing light-exposed dichromate which forms an image in an image-carrying layer of a hydrophilic, molecularly oriented, linear high polymer whereby to transform the dichromate to a dichroic material comprising iodine, said developing composition consisting of water, hydrochloric acid, at least one easily oxidizable, water-soluble iodide salt, an agent reactable with free iodine, and an agent comprising boric acid for controlling the color of the iodine image formed by development of said dichromate.

4. A composition for developing light-exposed dichromate which forms an image in an image-carrying layer of a hydrophilic, molecularly oriented, linear high polymer whereby to transform the dichromate to a dichroic material comprising iodine, said developing composition consisting of water, hydrochloric acid, at least one easily oxidizable, water-soluble iodide salt, a relatively weak alkali buffering said composition, a reducing agent, and an agent comprising boric

acid for controlling the color of the iodine image formed by development of said dichromate.

5. A composition for developing light-exposed dichromate which forms an image in an image-carrying layer of a hydrophilic, molecularly oriented, linear high polymer whereby to transform the dichromate to a dichroic material comprising iodine, said developing composition consisting of water, hydrochloric acid, at least one easily oxidizable, water-soluble iodide salt comprising ammonium iodide, an agent comprising boric acid for controlling the color of the iodine image formed by development of said dichromate, and an agent comprising a water-miscible liquid which is a non-solvent for the polymer of the image-carrying layer for slowing the penetration of the composition into the image-carrying layer.

6. A composition for developing light-exposed dichromate which forms an image in an image-carrying layer of a hydrophilic, molecularly oriented, linear high polymer whereby to transform the dichromate to a dichroic material comprising iodine, said developing composition consisting of water, an acid selected from the class consisting of hydrochloric, hydrobromic, sulphuric, nitric, phosphoric, and acetic acids, at least one easily oxidizable water-soluble iodide salt comprising ammonium iodide, an agent comprising boric acid for controlling the color of the iodine image formed by development of said dichromate, and an agent comprising a water-miscible liquid which is a non-solvent for the polymer of the image-carrying layer for slowing the penetration of the composition into the image-carrying layer.

EDWIN H. LAND.  
JOSEPH MAHLER.  
MARK HYMAN, JR.

#### REFERENCES CITED

The following references are of record in the file of this patent:

#### UNITED STATES PATENTS

| Number       | Name          | Date           |
|--------------|---------------|----------------|
| 1,214,940    | Miller        | Feb. 6, 1917   |
| 1,482,613    | John          | Feb. 5, 1924   |
| 2,059,884    | Mannes et al. | Nov. 3, 1936   |
| 50 2,059,887 | Mannes et al. | Nov. 3, 1936   |
| 2,141,354    | Gundelfinger  | Dec. 27, 1938  |
| 2,296,843    | Gaspar        | Sept. 29, 1942 |
| 2,396,726    | Trimble       | Mar. 19, 1946  |